

Dec. 29, 1970

A. COWEN ET AL

3,551,301

LEVELING HIGH SPEED PLATING

Filed April 14, 1966



Fig. 3



Fig. 4

INVENTORS

Arthur Cowen,  
Lynn T. Davies &  
BY Richard L. Teno

*L. J. Wallace*

ATTORNEY

3,551,301

## LEVELING HIGH SPEED PLATING

Arthur Cowen, Detroit, Lynn T. Davies, Pontiac, and  
Richard L. Teno, East Detroit, Mich., assignors to  
General Motors Corporation, Detroit, Mich., a corpora-  
tion of Delaware

Filed Apr. 14, 1966, Ser. No. 542,671

Int. Cl. C23b 5/02

U.S. Cl. 204—29

5 Claims

## ABSTRACT OF THE DISCLOSURE

Improving the leveling of electroplated, polished work-  
pieces by immersing the workpieces in a stream of flowing  
electrolyte and orienting the polishing grit lines at an  
acute angle to the direction of flow of the electrolyte.

This invention relates to high speed electroplating pro-  
cesses and more specifically to a method for improving  
the leveling characteristics of such processes.

Leveling can be defined as that property or characteris-  
tic of a plating solution or process which produces a sur-  
face smoother than that of the substrate. It is the usual  
practice to polish steel sheet before it is shaped into the  
desired part configuration. This polishing operation leaves  
extremely fine grit lines on the surface of the steel sheet  
that remain in the surface of the formed part. In order to  
get a perfect specular surface, as is needed for decorative  
chromium plating, these grit lines must be obscured. In  
the past this has been done by applying a heavy layer of  
copper or semibright nickel to the surface of the part be-  
fore the conventional bright nickel layer and chromium  
overlay are applied. If the copper or semibright nickel  
smooths out (levels) these grit lines, no buffing is required  
before the bright nickel layer and chromium overlay are  
applied. If insufficient leveling is obtained buffing is needed  
to smooth out the surface.

Some attempts have been made toward the direct adap-  
tation of organic bright nickel baths to improve leveling.  
Baths of this type are characterized by the addition of  
brighteners such as coumarin and its derivatives, acety-  
lenic alcohols, and nitrogen containing ring compounds  
such as pyridines, quinolines, and quaternary compounds  
such as pyridinium and quinolinium compounds. These  
techniques have been somewhat effective in conventional  
tank-type electroplating as well as the high speed electro-  
plating processes of this invention. High speed plating as  
used herein refers to those electroplating processes where  
the electrolyte is flowed past the workpiece at rates gen-  
erally in excess of 5 feet per second so as to permit satis-  
factory metal deposition at current densities up to and  
even in excess of 1,000 amperes per square foot (a.s.f.).

We have discovered a process which when used in con-  
junction with high speed plating processes will substan-  
tially reduce, and in most cases eliminate, the requirement  
for recourse to the prior art's prepolishing with subsequent  
buffing process steps.

It is an object of our invention to improve the leveling  
characteristics of high speed plating processes.

It is a further object of our invention to effect leveling  
in high speed plating processes by incorporating therein  
controlled workpiece orientation steps.

It is a further object of our invention to provide for  
the leveling of high speed electroplated coatings by a  
process which produces parallel polishing grit lines on the  
workpiece and then orients the workpiece in relation to  
the electrolyte flow so as to effect an angle between the  
polishing grit lines and the direction of electrolyte flow  
across the face of the workpiece. These and other objects

and benefits will become apparent from the following  
detailed description of but one specific embodiment en-  
compassed within the scope of our invention.

FIG. 1 is a partially sectioned elevational view of a  
device employing the invention.

FIG. 2 is a partially sectioned plan view of the device  
of FIG. 1 taken along section line 2—2 of FIG. 1.

FIG. 3 is a graphic representation of the benefits ob-  
tained by our invention.

FIG. 4 graphically compares high speed to conventional  
plating.

Briefly stated, our invention involves the improvement  
of the leveling capabilities already inherent in high speed  
electroplating processes and machines such as are dis-  
closed in copending U.S. patent application S.N. 212,318,  
High Speed Plating Method and Apparatus, filed July 25,  
1962. We improve these processes by polishing the work-  
piece, prior to plating, in substantially one direction, so  
as to leave substantially parallel grit lines on the surface.  
Subsequently the workpiece is oriented in the electrolyte  
flow channel so as to have the substantially parallel grit  
lines oriented at an angle to the direction of electrolyte  
flow across the face of the workpiece. While generally  
any acute angle between the orientation of the grit lines  
and the direction of electrolyte flow results in improved  
leveling, we have found that the larger acute angles  
approaching the perpendicular/transverse effect the great-  
est improvement (see FIG. 3).

Frequently the configuration of a particular part will  
not permit uniform unidirectional polishing. In these cases,  
polishing sequences or configurations should be so de-  
signed as to insure that the maximum portion of any sur-  
face can be polished in such a way as to present the maxi-  
mum grit line angle possible under the circumstances  
to the direction of electrolyte flow. Likewise since the  
important aspects of the invention lay in presentation of  
the workpiece to the electrolyte with its polishing grit  
lines at an angle greater than zero relative to the di-  
rection of electrolyte flow, it is immaterial what means  
are utilized to effect this end.

FIG. 1 is illustrative of the employment of our invention  
in a high speed electroplating device of the type  
disclosed in the aforementioned S.N. 212,318. The plat-  
ing device may consist of a tank 1 for holding an electro-  
lyte 2. The electrolyte 2 is circulated to the plating channel  
13 by means of pump 4. The electrolyte is pumped via  
conduit 3, through a screen or uniform flow control means  
5 and into plating channel 13. The electrolyte 2 flows  
between the nonconsumable lead anodes 11 and the work-  
piece 9. Workpiece 9, having grit lines 10, is passed into  
and through plating channel 13 by means of a holder 12,  
which is in turn a part of a channel sealing means or  
top 8. The top 8, and hence the workpiece 9, is moved  
from one channel to another in any desired plating se-  
quence by conveyor means extensions 15. The top 8 can  
have sealing means 16 to prevent loss of electrolyte.

The tank 1 may serve many purposes other than merely  
holding the electrolyte. It may, for example, be itself an  
electrolytic regeneration cell wherein the metal ion is re-  
plenished by the anodic dissolution of a pure metal elec-  
trode. It might also serve as a makeup mixing tank in  
addition to its function as an electrolyte holding tank.  
In effect, the only thing of significance here is that fresh  
nondepleted electrolyte be pumped from the tank 1 to  
the plating channel 13. How the electrolyte is replenished  
is not a part of this invention. Electrolytes for these  
systems are maintained fresh by any of a variety of  
known techniques, such as anodic dissolution replenish-  
ment, metal salt addition, and/or the like. As in sub-  
stantially all high speed electroplaters, the anodes 11 are  
of the fixed dimension nonconsumable type.

FIG. 3 shows one graphical representation of the leveling improvements that can be obtained by varying the angle of the grit lines to the electrolyte flow. As is clearly shown in FIG. 3, the most significant improvement was noted where the grit lines were at 73° to the direction of flow. For workpieces plated in accordance with our invention, leveling improvement in the order of 70% to 73% was observed. Percent leveling improvement is herein defined as,

$$100 \times \frac{(\text{orig. fin.}) - (\text{final finish})}{\text{original finish (RMS)}} = \text{percent}$$

For comparison purposes, similar samples were run concurrently with the test samples, varying therefrom only by having the grit lines parallel to the direction of electrolyte flow. The samples at zero grit line angle exhibited only 28% leveling. This 28% was felt to represent approximately the inherent leveling characteristic of high speed platers using electrolytes employing conventional brighteners. It is apparent therefore that under exactly the same conditions our invention has effected a 40% to 45% leveling improvement over the samples not prepared in accordance with our invention.

We have found that at a constant current density the leveling improvement begins even at flow rates in the order of 5 feet per second. As the flow rate is increased, the leveling improvement becomes more discernible.

We have found that the thickness of the plate contributes materially to the degree of improvement obtainable. Thus, FIG. 4 shows a comparison between the leveling improvement obtainable by high speed plating versus conventional plating as a function of the plate thickness required to effect a desired finish. We see, for example, that commencing with a 47 RMS finished sample, a 23.4% improvement (36 RMS) is possible with but 0.22 mil plate under high speed plating conditions whereas a like improvement under conventional plating conditions would require a 0.77 mil plate.

We have found as a practical matter that there are no significant advantages obtainable by usage of our process to improve samples having a surface finish rougher than 160 RMS. The time and thickness of plate required do not justify the efforts. Likewise, with starting samples having a roughness in excess of 160 RMS it is difficult to practically obtain final finishes much better than 18-20 RMS. In fact, there is a point above which the incident process will have no appreciable effect whatsoever. We know, for example, that a test sample displaying a roughness of 350 RMS could not be improved even with a 1.0 mil plate whereas the same sample was improved to 140 RMS with a 0.58 mil conventionally plated deposit. It is apparent, therefore, that somewhere between 160 RMS and 350 RMS there lay a point beyond which leveling improvement is practically impossible using this technique. Therefore, though we recognize that somewhat higher RMS surfaces than disclosed herein may be improved by our process, we find it impractical to do so.

#### EXAMPLE

Polished steel plates having an initial finish of 9-10 RMS were processed in accordance with the above comparison procedure.

The tests were conducted in a high speed plater of the type disclosed in the aforementioned copending application S.N. 212,318. A nickel bath containing 11.3 oz./gal. of nickel and 0.85 lb./100 gal. of Perflow was used. The bath was maintained within a pH range of 4.0 to 4.9 and a temperature range of 165° to 170° F. The electrolyte flowed across the surface of the respective samples at a rate of 45 to 50 feet per second. A current density of 1,000 amperes per square foot was applied for a total plating time of 76 seconds. The samples which were oriented at 90° to the direction of electrolyte flow in accordance with our invention displayed a 2-3 RMS final finish, whereas the samples maintained at zero grit line deviation displayed a 6-7 RMS final finish.

15 Though our invention has been described in terms of certain preferred embodiments, it is to be understood that others may be adapted and that the scope of our invention is not limited except by the appended claims.

We claim:

- 20 1. A process for effecting the leveling of electrodeposits in a high speed plating process comprising the steps of polishing the surface of a workpiece in substantially one direction so as to produce polishing grit lines substantially parallel to said one direction on said surface, cleansing 25 said workpiece, immersing said workpiece in an electrolyte, flowing said electrolyte across said surface, orienting said grit lines at an acute angle to the direction of flow of said electrolyte across said surface to improve the leveling of said electrodeposit, and passing current 30 through said electrolyte and said workpiece to effect metal deposition on said workpiece.
2. A process in accordance with claim 1 wherein said angle is from 62° to 90° inclusive.
3. A process in accordance with claim 1 wherein the rate of said electrolyte flow is at least about 5 feet per second.
4. A process in accordance with claim 3 wherein the metal is deposited for a time sufficient to produce a deposit of at least 0.22 mil thick.
- 40 5. A process in accordance with claim 3 wherein metal is deposited for a time sufficient to produce a deposit of at least 0.22 mil but not more than 1.0 mil thick.

#### References Cited

##### UNITED STATES PATENTS

- |           |         |                       |          |
|-----------|---------|-----------------------|----------|
| 1,886,218 | 11/1932 | Olin et al. -----     | 204—26X  |
| 3,007,854 | 11/1961 | Smith et al. -----    | 204—207X |
| 3,065,153 | 11/1962 | Hough et al. -----    | 204—237X |
| 3,071,521 | 1/1963  | Ehrhart -----         | 204—237X |
| 3,272,727 | 9/1966  | Schmeckenbecker ----- | 204—29   |
| 3,277,553 | 10/1966 | Wesolowski -----      | 204—29X  |

##### FOREIGN PATENTS

- |         |        |                     |         |
|---------|--------|---------------------|---------|
| 986     | 1896   | Great Britain ----- | 204—237 |
| 124,361 | 4/1945 | Australia -----     | 204—26  |

JOHN H. MACK, Primary Examiner

W. B. VAN SISE, Assistant Examiner